

## UNITED STATES PATENT OFFICE.

EDMOND DU BOIS, OF BASEL, SWITZERLAND, ASSIGNOR TO "CHEMICAL WORKS FORMERLY SANDOZ," OF BASEL, SWITZERLAND.

## PROCESS FOR INCREASING THE AFFINITY OF ANIMAL FIBERS FOR DYESTUFFS.

No Drawing. Application filed December 23, 1925, Serial No. 77,397, and in Germany January 6, 1925.

The present invention relates to a process for the treatment of animal fibers and has for its object to subject same to an operation which has the effect of increasing their affinity for dyestuffs of any kind, except the basic ones. This refers not only to dyestuffs, which, without such a treatment do not possess any affinity, but also to those, which commonly are absorbed by the animal fiber, whereby in the latter case, an important increase of the affinity is obtained.

The process consists in a suitable treatment of the fibers with esterifying agents, whereby this treatment can be effected in any working state of the fiber.

To perform the process, the following esterifying agents may enter into consideration: halides of aliphatic, aromatic and alicyclic carboxylic and sulphonic acids, as well as aromatic anhydrides. Such a treatment has the effect of considerably increasing the affinity of acid dyestuffs.

The following examples illustrate the improved process.

*Example 1.*

20 g. of wool are thoroughly worked for two hours at 40-50° C. within 250 g. of a 20% solution of paratoluolsulphone chloride in toluene, then squeezed out or hydroextracted and washed at 60-70° C. consecutively with several weak soap solutions. Thereupon the fibers are rinsed with cold water for some time and dried.

The fibers thus treated show a considerably increased affinity compared to the untreated ones, they can further be dyed to a large extent with direct cotton dyestuffs, whereby it is possible to dye in a neutral bath without any addition. The dye-bath is exhausted in a much shorter time than by untreated wool.

*Example 2.*

20 g. of wool are worked for two hours very thoroughly within a suspension of 30 g. of para-toluol-sulphone chloride, finely pulverized, and 20 g. of chalk in 250 g. of water at 75° C. and afterwards subjected to the after treatment as indicated in Example 1. The tinctorial properties of the fiber thus obtained are identical to those of Example 1.

*Example 3.*

20 g. of wool are treated, as indicated in

Example 1 with 250 g. of a 20% solution of benzoylchloride in toluene, then washed in the weak soap solutions as stated, subsequently rinsed and dried.

The increase of affinity for all acid dyestuffs in a neutral bath is very distinct, also direct cotton dyestuffs dye the fiber to a large extent.

*Example 4.*

20 g. of wool are treated with 250 g. of a 20% solution of acetylchloride in toluene, as indicated in Example 1, and then after treated in the same manner as above. The fiber thus obtained shows the tinctorial properties as stated in Example 1.

*Example 5.*

20 g. of wool are worked for two hours very thoroughly within a suspension of 50 g. salicylic acid sulphone chloride in 200 g. of toluene at 60° C. and then after treated according to Example 1. The fibers thus obtained show a strongly increased affinity for acid dyestuffs; they are also dyed to a particular extent with direct cotton dyestuffs.

*Example 6.*

20 g. of wool are worked thoroughly for two hours within 250 g. of a 20% solution of benzoic acid anhydride in toluene and then subjected to the after treatment as indicated in Example 1. The tinctorial properties of the fibers thus obtained are identical to those of Example 1.

*Example 7.*

20 g. of wool are treated according to the indications of Example 1 with 250 g. of a 20% alcoholic solution of phthalic acid anhydride and then after treated as stated in the first example. The tinctorial properties of the fibers thus obtained still surpass those described in Example 1.

What I claim is:—

1. A process for increasing the affinity of animal fibers for dyestuffs, consisting in treating the animal fibers with acylating agents.

2. A process for increasing the affinity of animal fibers for dyestuffs, consisting in treating the animal fibers with aromatic acylating agents.

3. A process for increasing the affinity of

animal fibers for dyestuffs, consisting in treating the animal fibers with halides of aromatic sulphonic acids as esterifying agents.

5. A process for increasing the affinity of animal fibers for dyestuffs, consisting in treating the animal fibers with chlorides of aromatic sulpho acids.

5. A process for increasing the affinity of animal fibers for dyestuffs, consisting in treating the animal fibers with para-toluol-sulphone chloride as esterifying agent and then washing same with weak soap solutions.

In witness whereof I have hereunto signed my name this 7th day of December, 1925.

EDMOND DU BOIS.